# EUROPEAN PATENT APPLICATION

(11) **EP 0 668 219 A1**
(43) Date of publication of application: **23.08.1995**
(21) Application number: 95100847.3
(22) Date of filing: 23.01.1995
(51) Int. Cl.: B65D 65/42

(54) **A plastic package possessing superior barrier properties**

(30) Priority: 04.02.1994 CH 325/94
(71) Applicant: TETRA LAVAL HOLDINGS & FINANCE SA, 1009 Pully (CH)
(72) Inventor: Frisk, Peter, D-6104 Seeheim-Jugenheim (DE); Roulin, Anne, CH-1415 Molondin (CH); Jaccoud, Bertrand, CH-1678 Siviriez (CH); Johansson, Hans, D-65835 Liederbach (DE)
(74) Representative: Sundell, Hakan

(57) **Abstract**

The disclosure relates to a package of plastic with a layer, applied on the inside of the package, of a silicon oxide compound of the general chemical formula SiOₓ, where x may vary from 1,8 to 2,2.

The thin silicon oxide layer which is produced by vacuum deposition direct on the inner surfaces of the package has a thickness of less than 2000 Å.

At the same time as the silicon oxide layer of the package efficiently prevents migration of foreign components or substances into a product which is packed in the package, it also displays superior barrier properties against absorption or other take-up of flavour and aroma substances occurring in the product, so-called non-scalping properties.

## Description

### TECHNICAL FIELD

The present invention relates to a package for the distribution of foods and more precisely relates to such a package as possesses superior barrier properties.

### BACKGROUND ART

These days, foods such as milk, juice etc. are most generally packed and transported in packages of a single-use disposable nature, i.e. packages which are intended to be used only once and then disposed of. Examples of such disposable packages are the common milk or juice cartons of plastic-coated paper which, after use, are collected and destroyed at some central plant for waste management.

There are also ready-to-consume portion or user packages of multi-use type available on the market and these, after the first use, are intended to be re-used for new distribution of foods. Examples of such multi-use packages are bottles of plastic or glass which are often employed for packing and transporting soft drinks and similar ready-to-drink beverages.

While the single-use disposable packages are both easy to produce and handle and, in addition, more than satisfy those demands which are placed on acceptable protection and good shelf-life for the packed product, the multi-use packages constitute an attractive complement or alternative which, at least from the point of view of materials savings, enjoys a number of advantages over single-use packages.

However, one disadvantage inherent in multi-use packages is that, prior to each occasion of re-use, they require meticulous cleaning, with consequential consumption of washing and rinsing solutions and the related consumption of chemicals and energy. A further disadvantage is that multi-use packages become worn with use and lose their pristine appearance as a result of the mechanical stresses to which the packages are subjected during transport and other handling. Yet a further disadvantage is that packages produced from plastics, e.g. plastic bottles, may contain components which tend to migrate into and taint the product contained in the filled package.

### OBJECTS OF THE INVENTION

One object of the present invention is, therefore, to obviate the above-outlined drawbacks inherent in the prior art technology.

A further object of the present invention is to devise a multi-use package for distribution of foods, without the intimately related drawbacks of the type described in the foregoing.

Yet a further object of the present invention is to devise a multi-use package which, after use, is easy to clean and prepare for re-use, without consuming washing and rinsing solutions with the associated chemicals, as in the prior art technology.

Still a further object of the present invention is to devise a multi-use package possessing superior barrier properties against migration of components or substances of a foreign nature present in and/or on the walls of the package into the product packed therein.

Yet a further object of the present invention is to devise a multi-use package possessing not only superior barrier properties against migration of such components and substances but also superior barrier properties against gases such as oxygen gas.

Still a further object of the present invention is to devise a multi-use package possessing superior non-scalping properties, i.e. a multi-use package which, in itself, does not absorb or otherwise take up flavour or aroma substances present in the packaged product.

### SOLUTION

These and other objects and advantages will be attained according to the present invention by a multi-use package of the type which is defined in appended Claim 1.

Expedient and preferred embodiments of the multi-use package according to the present invention have further been given the characterizing features as set forth in the appended subclaims.

### DESCRIPTION OF PREFERRED EMBODIMENT

According to the invention, it has proved that a multi-use package, for example a bottle of plastic produced by blow moulding may, in a simple manner and by simple means, be provided with a coating of a silicon compound which, by so-called vacuum deposition, is deposited on the inside of the package for the formation of a thin continuous coating of the above-mentioned silicon compound.

The expression "vacuum deposition" (which is well-known to a person skilled in the art) is here taken to signify conventional deposition techniques such as plasma deposition, vapour deposition, chemical plasma vapour deposition, sputtering etc., which constitute examples of such known deposition techniques.

The preferred vacuum deposition technique according to the present invention is chemical plasma vapour deposition, abbreviated to CPVD, which makes it possible to produce extremely thin but nevertheless extremely tight continuous coatings which, with good adhesion, bond to the inner walls of a previously produced package, e.g. a plastic bottle, according to the invention.

By the chemical plasma vapour deposition method (CPVD), it is possible to deposit such thin, continuous coatings of a silicon compound of the general chemical formula SiOₓ (where x may vary from 1,8 to 2,2), which has proved to be that silicon compound which is most preferable and advantageous for the purposes of the present invention. Such a coating of an SiOₓ compound which, according to the invention, is of a thickness of less than 2000 Å, possesses excellent adhesive capability to the package walls and is mechanically strong and durable, at the same time as it possesses excellent barrier properties against migration of foreign components or substances and, in addition displays superior gas barrier properties without, in itself, absorbing or otherwise taking up flavour or aroma substances which occur in certain types of foods such as, for example, citrus juices.

The thickness of the applied silicon oxide coating is, as intimated above, less than 2000 A and is ultimately determined by that type of product which is to be packed and transported in the package. In general, the thickness is such that the coating will be easily dissolved and removed during washing, e.g. less than 2000 Â. If the package is to be employed for products ultra-sensitive to gas (for example sensitive to oxygen gas) which are rapidly broken down or deteriorate in quality in contact with gases, the coating is made thicker within the disclosed thickness range, while less sensitive products require considerably thinner coatings. Since the chemical plasma deposition technique makes possible a switch from one thickness to another, it is, thus, easy to "tailor make" the applied coatings for optimum adaptation to a given product on every occasion.

A multi-use package according to the present invention may, after use but prior to the next filling, readily be provided with a new coating (once the first coating has been removed) by vacuum deposition, preferably chemical plasma deposition, which is repeated every time the package is to be refilled, if necessary. The advantage inherent in applying a new coating prior to each product filling is that the returned, empty package requires no careful cleansing operation to the extent necessary when employing prior art multi-use packages.

The present invention will be described in greater detail hereinbelow, with particular reference to one example, chosen merely by way of non- restrictive exemplification, of a multi-use package according to one preferred embodiment of the invention. The described example should, hence, not be perceived as restrictive of the scope of the present invention which, without departing from the spirit and scope of the general description and subsequent Claims, also encompasses modifications and variations obvious to a person skilled in the art.

A prefabricated bottle of plastic (e.g. polyester, polycarbonate, polypropylene, polyethylene, polyamide or polyethylene naphthenate) produced in a conventional manner (for example by blow moulding techniques) is placed in a vacuum chamber arranged for vacuum deposition in accordance with the chemical plasma deposition technique and is coated on its inner walls with a thin coating of a silicon oxide compound of the general chemical formula SiOₓ, where x may optionally vary from between 1,8 to 2,2. During the deposition process, the formed silicon coating is deposited direct on the inner walls of the bottle for the formation of a progressively growing layer or stratum which covers the entire inside of the bottle. The process is discontinued when the deposited stratum has reached a predetermined thickness which is less than 2000 Å, depending upon what type of product the bottle is intended for. After completed coating operation, the coated bottle is removed from the vacuum chamber and is conveyed to a product filling plant where the bottle is filled, with the aid of a conventional filling machine, with the pertinent product for further distribution to a point of consumption or retail outlet.

When the bottle has been emptied of its contents, the emptied bottle is returned for re-use, whereupon it (possibly after cleaning and removal of the earlier coating) is provided with a new inside coating in the above-described manner and is thereafter filled with new product which may be, but not necessarily is, the same product as before.

It will be apparent from the foregoing description that the present invention makes possible, by simple conventional technology, an efficient and product-safe re-use of packages.

Even though the present invention has been described with particular reference to a package of the bottle type, other forms of packages may naturally be employed, such as cans, beakers and other geometrically regular or irregular cup-shaped package configurations. In addition, the package according to the present invention need not be produced from plastic or by means of the above-mentioned blow moulding technology, but other packaging materials and production methods known in the art are possible and applicable without departing from the spirit and scope of the inventive concept as herein defined by the appended Claims.

## Claims

1. A package possessing superior barrier properties, characterized in that it has, on its inner walls, a coating of a silicon compound of the general chemical formula SiOₓ, where x may vary from between 1,8 and 2,2, and in that said coating is produced by chemical plasma vapour deposition in a per se known manner.

2. The package as claimed in claim 1, characterized in that the coating is disposed to cover the entire inside of the package.

3. The package as claimed in claim 1 or 2, characterized in that the coating is disposed for direct contact with a product packed in the package.

4. The package as claimed in any one of the preceding claims, characterized in that it substantially consists of polymer.

5. The package as claimed in any one of the preceding claims, characterized in that the thickness of the coating is such that the coating will be easily dissolved and removed during washing, e.g. less than 2000 Å.
